

Aug. 4, 1959

R. F. STUEWER

2,897,577

## METHOD OF DULLING NYLON AND LIKE MATERIALS

Original Filed May 12, 1954

7 Sheets-Sheet 1

上古文



## INVENTORS

Reinhold F. Stuewer

BY

Mason, Porter, Diller & Stewart,

ATTORNEYS

Aug. 4, 1959

R. F. STUEWER

2,897,577

METHOD OF DULLING NYLON AND LIKE MATERIALS

Original Filed May 12, 1954

7 Sheets-Sheet 2



Reinhold F. Stuewer

BY *Mason, Porter, Diller & Stewart,*

ATTORNEYS

Aug. 4, 1959

R. F. STUEWER

2,897,577

METHOD OF DULLING NYLON AND LIKE MATERIALS

Original Filed May 12, 1954

7 Sheets-Sheet 3



BY *Mason, Porter, Dillon & Stewart,*

ATTORNEYS

Aug. 4, 1959

R. F. STUEWER

2,897,577

METHOD OF DULLING NYLON AND LIKE MATERIALS

Original Filed May 12, 1954

7 Sheets-Sheet 4



BY Mason, Porter, Dillon & Stewart,

ATTORNEYS

Aug. 4, 1959

R. F. STUEWER

2,897,577

METHOD OF DULLING NYLON AND LIKE MATERIALS

Original Filed May 12, 1954

7 Sheets-Sheet 5



BY *Mason, Porter, Dillon & Stewart,*

ATTORNEYS

Aug. 4, 1959

R. F. STUEWER

2,897,577

## METHOD OF DULLING NYLON AND LIKE MATERIALS

Original Filed May 12, 1954

7 Sheets-Sheet 6



INVENTORS

Reinhold F. Stuewer

BY Mason, Porter, Dillon & Stewart,

ATTORNEYS

Aug. 4, 1959

R. F. STUEWER

2,897,577

METHOD OF DULLING NYLON AND LIKE MATERIALS

Original Filed May 12, 1954

7 Sheets-Sheet 7



INVENTORS

Reinhold F. Stuewer

BY Mason, Porter, Della & Stewart,

ATTORNEYS

## 1

2,897,577

METHOD OF DULLING NYLON  
AND LIKE MATERIALS

Reinhold F. Stuewer, Scranton, Pa., assignor to Grove Silk Company, Scranton, Pa., a corporation of Pennsylvania

Original application May 12, 1954, Serial No. 429,244.  
Divided and this application April 11, 1955, Serial No. 500,630

## 14 Claims. (Cl. 28—72)

This invention relates to an art of performing dulling operations upon the surfaces of fibers such as nylon. The extruded and set fibers of synthetic fibers, whether in filament or cut staple form, frequently are too smooth and shining for satisfactory appearance and behavior. The present invention is concerned with a superficial treatment of such fibers to confer a desired dullness or matte appearance thereto, in economical quantity operations.

This application is a division of the Stuewer and Pittman application Ser. No. 429,244, filed May 12, 1954.

A feature of the invention is that of holding a yarn of such fibers under tension and for causing the fibers to be pressed in contact with particles of an indenting material.

Another feature is that of treating skeins of such yarn by holding them under tension along the fibers while kneading the yarn in the presence of particles of an indenting material.

A further feature is that of holding a skein of such yarn under tension, and yieldingly pressing against the yarn while causing the skein to travel through the pressure zone and thereat be subjected to relative movements of the fibers with particles of an indenting material between them.

Other features reside in the performance of a sequence of operations whereby the fibers are converted from a smooth to a dulled surface condition, without entanglement.

An illustrative embodiment of apparatus by which the method may be performed is shown on the accompanying drawings, by way of example, in which:

Fig. 1 is an upright elevation of the left side of machine structure;

Fig. 2 is a corresponding front elevation with a part broken away;

Fig. 3 is a corresponding elevation of the right side of machine structure;

Fig. 4 is an enlarged horizontal section substantially on line 4—4 of Fig. 2 with the door open and the upper skein-guiding roller and spray pipe in position for loading or unloading;

Fig. 5 is a corresponding horizontal section substantially on line 5—5 of Fig. 2 with the door omitted and the lower skein-guiding roller being swung to position for loading and unloading;

Fig. 6 is an upright sectional view on an enlarged scale, substantially on line 6—6 of Fig. 2;

Fig. 7 is a conventionalized perspective view, with supporting and certain other parts omitted for clarity, showing the relationship and connection of parts;

Fig. 8 is a diagrammatic view, with parts of a control system in perspective, showing electrical connections.

Commercially available fibers contain synthetic materials such as polyamides, and are formed by an extrusion operation from a mass, with subsequent setting followed by a stretching operation which produces orientation within the individual filaments. Sometimes the original

5

## 2

mass contains a pigment to reduce the light transmission, and the material is then referred to as a "semi-dull" or "dull" dependent on the relative amount of pigment present; but the surface of the material is still essentially smooth as with the non-pigmented or "bright" filaments.

Such fibers may be used as monofilaments, or several filaments may be twisted together; and a further practice is to cut the filaments into lengths and spin together in cut staple form. The present invention is applicable to the various forms and sizes, and produces an effect distinct from that attained by incorporated pigment.

For illustrative comparison of sizes, it may be stated that nylon yarns are presently commercially available and used in quantity for stockings and knit goods in the following typical sizes:

| Denier | Filament Count | Diameter of Filaments in Microns |
|--------|----------------|----------------------------------|
| 40     | monofilament   | 73                               |
| 15     | do             | 44                               |
| 12     | do             | 39                               |
| 40     | 13 filament    | 19.5                             |
| 70     | 34 filament    | 16                               |
| 20     | 20 filament    | 11.5                             |

The main mechanical structure is supported by four pipe legs 20 connected by welding to angle irons 21 and a front iron 22 providing a horizontal stand upon which is mounted a housing having the side walls 24, 25 and the rear wall 26. The lower part of the front of this housing can be closed by a door 28 on hinges 29 and having a latch 30 for securing it in closed position; it is preferred to have the lower edge 31 of the door bent inwardly so that liquid is deflected inside of the front iron 22 and delivered into the catch basin or sump 8 which is conventionally shown as a liquid-tight box mounted on wheels 33 so that it can be withdrawn through the front pair of legs 20, its position being controlled by the front stiffener 34 which extends upwardly and engages the front iron 22.

At the top of the housing formed by walls 24, 25, 26 is mounted a control housing CH described in detail hereinafter. Also mounted at the top of the housing 24, 25, 26 are a pair of upwardly extending pipes 35 which are held rigidly in upright position by straps 36.

At the left side of the machine (Figs. 1 and 4) a horizontal supporting member 38 extends from the wall 26 and is connected to the upright member 39 to provide support for valve and pipe structures as described hereinafter. Angle braces 40 likewise serve to brace the pipe connections.

This frame structure supports the moving parts.

The walls 24, 25 have pivots 42 for supporting the lever arms 43 of a rocking sub-frame, these arms being outside of the walls 24, 25 and supporting the shaft 44 of a lower pressure roller 45 having a smooth rubber covering 46 (Fig. 6). The shaft 44 can move upward and downward in the elongated apertures 47 of the walls 24, 25. The shaft 44 has connected thereto the sprockets 48 which in turn are connected by chains 49 with the sprockets 50 carried by the rear driving shaft 51 which passes through a speed reduction unit 52 which illustratively is of commercial type and has a shaft 53 extending rearwardly and supporting a pulley 54 for belt 55 which is driven by pulley 56 of the driving motor DM. This motor DM is supported by struts 57 connected to a crossplate 58 rigid with the arms 43. It will be noted that the weight of the motor and its struts, the weight of the reduction unit, and the bearing parts act to cause the sub-frame to rock clockwise in Figs. 3 and 6, about the pivots 42, thus moving the lower pressure roller 45

upwardly; and that this pressure can be increased by the employment of a predetermined number of removable weights 59 which are held against shifting by the securing bolts 60.

The rocking sub-frame can be rocked in an opposite direction by the cams 65 (Fig. 6) which are fixed on a cam shaft 66 journaled on the support irons 21 and having (Fig. 3) a worm wheel 67 presented for meshing engagement with the worm 68 on a shaft 69, likewise carried by bearings on the irons 21 and on the posts 20, and having a crank handle 69a at the front of the machine.

The left-hand housing wall 24, in the illustrated form, supports a swivel bearing 70 (Figs. 1 and 5) for the end of a second pressure roller 71 which likewise has a smooth surface jacket 72 of rubber. This bearing 70 permits the roller 71 and its jacket 72 to rotate, and also permits it to be swung (Fig. 5) out of the housing. When swung back into operating position, the right-hand end of the shaft 73 of the roller engages in a notch 74 formed in the wall 25 (Fig. 3); and its axis is then parallel to the axis of the lower pressure roller and the shaft 44 of the latter. In this working position, the weights on the sub-frame cause the arms 43 to rock clockwise so that the lower pressure roller 45 is in contact with the second pressure roller 71 or with yarn skeins passing therover, the lower roller being thus yieldingly mounted.

Within each of the pipes 35 is provided a coil spring 80 (Fig. 6) which is mounted at its upper end on a threaded stem 81 extending through the end cap 82 of the pipe and adjustable in position by the nut 83. The lower end of the spring is connected to a drag link 84 which in turn is connected to a bearing 85. The two bearings 85 support the shaft 86 of an upper tension roller 87 which may have a smooth metal surface. A bracket 88 extends forwardly from the housing wall 24 and has a sleeve member 89 fixed thereon for receiving (Fig. 4) the left-hand end of the shaft 86 when the parts are in position for loading, noting that the bracket 88 is located below the normal level of the shaft 86 (Fig. 6) when the latter is in its tensioned operating position.

The support 38 (Figs. 1 and 4) carries three valves 90, 91, 92 which are connected to a manifold pipe 93 supported in part by the angle braces 40 and leading to the distributing pipe 94 from which extends a horizontal spray pipe 95 located (Fig. 6) just inside of the rear wall 26 of the housing and having orifices directed relatively downward and forward for delivering a liquid spray 97 as described hereinafter. The distributing pipe 94 is also connected through a swivel joint 98 with a second spray pipe 99 which terminates short of the end wall 25 of the housing, so that it may be swung (Fig. 4) out of the housing during loading and unloading operations.

Limit fingers 100 are provided for preventing disengagement of skeins during the loading operation, being illustratively supported by the back wall 26. Preferably the spray pipe 99 has upwardly and rearwardly directed openings so that a liquid spray 101 is delivered therefrom as described hereinafter.

The door 28 has separators or guide fingers 105 fastened on its rear or inner wall (Figs. 4 and 6), and thus projecting between skeins of yarn when the door is in closed position.

The housing CH at the top of the structure has a tightly-closing access door 110 at its front, and contains and protects electrical elements that determine a sequence of operations.

In Figs. 7 and 8 are shown conventionalized parts of the structure connected to illustrate the operation. A supply of satisfactorily pure water under pressure is delivered through a pipe 120 to the valve 90. A soaping solution is prepared in a soap solution tank ST having a motor-driven pump STP connected for taking the solution from the tank and delivering it through a hose 121

75 to the valve 91. Correspondingly, an oil emulsion is prepared in an oil emulsion tank OT having a motor-driven pump OTP which takes the oil emulsion from the tank and delivers it through the hose 122 to the valve 92. The valves 90, 91, 92 have respective solenoids WVS, SVS and OVS which upon energization serve to open the respective valves.

A timing motor TM is connected through speed reduction gearing 125 to drive a timing shaft 126 having thereon a number of cams MC, WC, SC, OC and RC cooperative with corresponding switches MS, WS, SS and OS which are normally open but are closed upon presentation of a cam notch, and a switch RS which has both normally open and normally closed contacts selectively closed and opened by the notches and humps on cam RC. The master cam MC has illustratively a single peripherally short notch for operating the master switch MS. A manual switch S1 is connected in parallel to switch MS, so that when switch S1 is closed current flows from one mains conductor 130 through the mains switch S2 and the switch S1 to the bus conductor 131 thereby energizing the timing motor TM so that it runs; the current then returning to the other mains conductor 132. As the timing motor rotates the shaft 126, the master cam MC operates switch MS and closes the circuit so that the flow from conductor 130 to bus conductor 131 is maintained regardless of the position of switch S1, which is then permitted to open.

In the illustrative showing, a 15 minute cycle of operation is established by the gearing 125, so that the motor TM rotates the shaft 126 once in 15 minutes. At the beginning of rotation of the shaft 126 only the master switch MS is in operation, and therewith the reversing cam RC is holding the reversing switch RS with one circuit open and the other circuit closed through the conductors 133, 134 leading to the coils of the reversing relays RR<sub>a</sub>, RR<sub>b</sub> so that current from the mains conductors 130, 132 flows through a relay RR<sub>a</sub> or RR<sub>b</sub> and by conductors 140 to the driving motor DM, causing this motor to start and turn in one direction. The relays RR<sub>a</sub> and RR<sub>b</sub> are mechanically interlocked, as conventionalized by the element RR<sub>x</sub>, so that they cannot be simultaneously energized: such grouped relays are commercially available and no further detail of structure or operation need be given to the electrical expert. At an interval thereafter, determined by the spacing of the multiple cam depressions in reversing cam RC, the switch RS acts to open and close the circuits of the conductors 133, 134 so that the other reversing relay RR<sub>b</sub> or RR<sub>a</sub> is actuated whereby the driving motor DM is then caused to run in a reversed direction for another period of time until the reverse cam RC acts again. Illustratively, this reversal occurs at each 30 seconds of time, with the motor DM thus turning for 30 seconds in one direction and then turning for 30 seconds in the opposite direction.

In the illustrative cycle, the water controlling cam WC has two depressions, the first of which procures operation of the water controlling switch WS after the shaft 126 has been rotated for a distance corresponding to 10 minutes and 30 seconds of time, closing the normally open contact of this switch so that current flows from the bus 131 through switch WS to conductor 135 and thus to the water valve solenoid WVS, opening the valve 90 so that water flows from the conduit 120 through the manifold 93 and is sprayed from the pipes 95, 99 upon the skeins of yarn which are passing over the tension roller 85 and the uppermost pressure roller 71. In this illustrative cycle, the length of this first depression on cam WC effects the valve opening for 10 seconds, and the water serves to moisten the thickened slurry present in the yarn. Thereupon, the depression leaves the switch WS, and the switch is opened again, therewith the valve 90 is closed.

Immediately following the wetting operation just described, the soap solution cam SC presents its single de-

pression to its switch SS, with closing of the normally open contact thereof, so that current flows from the bus conductor 131 through the switch SS and by conductor 136 to the solenoid SVS thereby opening the valve 91 so that the soap solution is permitted to flow from the conduit 121 through valve 91 and manifold 93 and be sprayed from the pipes 95, 99. In the illustrative cycle, this continues for 10 seconds, and the cam SC then opens the switch SS again, thereby effecting closure of the valve 91.

Thereafter, for 2 minutes, the master switch MS acts in conjunction with the reversing switch RS to cause the driving motor DM to continue running for 2 minutes, with the aforesaid periodic reversal being accomplished by the action of switch RS upon the current supply to the relays RR<sub>a</sub>, RR<sub>b</sub>.

After 2 minutes of running with the soap solution in the fibers, the second depression on the water supply cam WC is presented to the switch WS which closes, and current again flows through conductor 135 to the water valve solenoid WVS, and valve 90 opens again and remains open for 2½ minutes, wherewith water flows from the conduit 120 to the manifold 93 and the spray pipes 95, 99; and the abrasive material is washed from the yarn fibers. During this time, the switches MS, RS are in control of the driving motor DM, so that the same continue to run with the aforesaid periodic reversal.

Thereafter, the cam OC which controls the delivery of oil emulsion presents its single short depression to the oil emulsion controlling switch OS, with closing of the contact therein so that current flows by conductor 137 to the solenoid OVS of valve 92, and the valve 92 opens so that the oil emulsion in conduit 122 flows through valve 92, manifold 93, and from the spray pipes 95, 99, wherewith the fibers are oiled. After this has continued for 10 seconds, the cam OC causes the switch OS to open again, and the valve 92 closes. Simultaneously, the single depression in the master cam MC cooperates with the master switch MS to open this switch, so that current no longer flows from mains conductor 130 and bus conductor 131 and the timing motor TM stops: simultaneously, supply of current to the various switches WS, SS, OS, and RS fails, so that accidental operation of the solenoids WVS, SVS, OVS cannot occur, and also the reversing relays RR<sub>a</sub>, RR<sub>b</sub> remain in open positions so that the motor DM is brought to and held at a standstill.

It is preferred, for operation of a single machine from the soap solution and oil emulsion tanks ST, OT, to connect the respective pump motors to the conductors 136, 137, so that the pump motors STP, OTP are operated concurrently with the opening of the valves, nicety of control being effected by the quick action of the valves 91, 92 in closing.

To permit quick stoppage of the system if desired, a manual switch S2 is provided in the conductor 130.

In operation of the machine, with the machine empty, an abrasive slurry is prepared and skeins of yarn dipped and worked therein for receiving charges. The upper tension roller is removed from its bearings 85, and the left-hand shaft end 86 is introduced into the holding bracket 89, with the door 28 open (Fig. 4). The spray pipe 99 is swung outwardly to the position of Fig. 4. The lower pressure roller 45 is moved downward by turning the crank 70 so that cam 65 (Fig. 6) engages the bottom of the sub-frame structure 43, 58 and lifts the same: thus relieving pressure from the upper pressure roller 71. The upper pressure roller 71 is then swung outward about its bearing 70 to the position of Fig. 5. Skeins of yarn are then threaded onto the rollers by passing them around the tension roller 87, the spray pipe 99, and the pressure roller 71, arranging them closely against one another along the length of the tension roller 87, wherewith the left-hand finger 100 serves to prevent these skeins from being moved beyond the ends of the

rollers. In the illustrative practice, with rollers having a length of 24 inches, 24 skeins of the commercial 2 ounce size are employed. The pressure roller 71 is then swung back into the housing and engaged in the notch 74, carrying the lower ends of the skeins with it. The upper or tension roller 87 is taken from the bracket 88, 89 and its ends engaged in the bearings 85 which can be pulled downward and outward for the purpose: upon release of the traction links 84, a tension is established in the skeins of yarn as these are stretched upward by the movement of the tension roller 87 upward and away from the pressure rollers, the skeins being controlled against endwise shifting by the fingers 100 supported from the rear wall 26 at about one inch from the end planes of the rollers. The spray pipe 99 is swung into its position of use (Fig. 6).

The door 28 is now moved toward closed position, until its guide members 105 approach the skeins of yarn. By hand, the left-hand four skeins are separated so that their outer and downward flights, at the left in Fig. 6, come between the first two guide members 105. The next four skeins are likewise parted so that they come between the second and third guide members 105 and so forth. The door is partly closed at each separation, so that the skeins are held. The door is closed and latched. It will be noted that this latter operation is facilitated in that the upper edge of door 28 is below the position of fingers 100, so that a substantial part of each skein is accessible above the door edge.

The crank 70 is again rotated so that the cams 65 release the rocking sub-frame, and the pressure roller 45 is permitted to move upwardly under the weight imposed by the driving motor DM, and other parts of this sub-frame, until it comes in yielding engagement with the skeins at their lower flights, and forces these against the pressure roller 71.

The cycle of operation is then started by closing the switch S1, and the operation occurs as described above, wherewith the rotation of the driving motor DM causes the lower pressure roller 45 to be rotated while in contact with the skeins of yarn, so that the same are caused to travel; during the counterclockwise rotation of the roller 45, the outer or front flight of the skeins of yarn moves in an upward direction, and upon reversal, with the clockwise rotation of the roller 45, the outer or front flight moves downward in Fig. 6. The lower pressure roller 45 yieldingly presses the yarn against the upper pressure roller 71, and the latter turns. The tension upon the skeins may be regulated by adjusting the nuts 83.

During the described cycle, the driving motor DM operates for 10½ minutes, with reversal of direction every 30 seconds, and during this time the kneading effect of the rubber-covered pressure rollers 45, 71 upon the fibers in the skeins causes these fibers to move relative to one another with the abrasive particles therebetween and indentation is produced upon the surfaces of the fibers but with no significant wearing away or gouging out of material. During this action, the water vehicle of the slurry is partly squeezed out and drops into the sump S; wherewith the initial action is in the presence of a greater amount of moisture than the action toward the end of the period. Thereupon, water is admitted for 10 seconds to restore wetness to the passing yarn, followed by the delivery of a soaping solution for 10 seconds and then running in the presence of the soap solution for 2 minutes, wherewith the particles become loosened if embedded in the surface of the fiber. Thereafter, a continued running occurs with a water spray for 2½ minutes, resulting in the washing of essentially all particles from the yarn. In each phase of operation, the liquid flows downward and enters the sump S. Finally, an oil emulsion is delivered for 10 seconds, therewith coating the fibers and permitting, after drying, of knitting these oiled fibers without difficulty.

As the motor DM turns in a clockwise direction, for example, the relative movements of the fibers as they pass between the pressure rolls 45, 71, and the difference in length between the turns of yarn at the inner and outer sides of a skein, tend to cause irregularity or bunching: but the following reversal compensates for establishing a proportioned correcting effect in the opposite direction: and in practice it has been found that the yarn can be unwound from the skeins without difficulty.

Among the materials satisfactory in particle form are powdered calcite, very finely powdered glass and diatomaceous earth. Fine sodium bicarbonate crystals have been employed and, in general, any insoluble or limitedly-soluble material of proper particle size may be used, which has the hardness property of producing the indentation. In general, materials having a hardness of 2 or more on the Moh scale can be used, for example finely ground rock salt or harder substances; with dominant preference for materials in particles having sharp corners or edges. Diatomaceous earth has been found highly satisfactory for the dulling or delustering operation, and the observation has been made that the particles are broken up and comminuted during the treatment.

The hardness of such appropriate materials cannot be directly compared to the hardness of nylon, for the reason that the nylon behaves somewhat like a metal in having ductility and capability of being dented, and also has an elastic rubbery quality. For example, when two 40 denier monofilaments of nylon are crossed and pressed between two glass plates, each is flattened at the intersection until its dimension decreases in the direction of the pressure and its dimension transverse to the pressure increases 50 percent: when the pressure is released, each filament tends to regain its shape, for example losing half of the transverse increase in diameter. Thus a Brinell test for hardness of nylon gives an exaggerated result as compared with a Rockwell test. As further examples of behavior, if an unstretched mass of nylon plastic is pressed by a needle point, a depression is formed with a raised rim around it, which recedes partially when the needle is removed; and if the needle is drawn along the surface, under pressure, a furrow is formed with a central groove and raised edges but no material is removed. Likewise, pressing a layer of fine rocksalt crystals against an originally smooth and shining surface of a block of unstretched nylon causes indentation, but without removal of material even if the crystals are displaced by rubbing; and the surface after removal of the material exhibits loss of the original shine. It is to be remarked, further, that nylon filaments have been stretched during manufacture, and have attained an oriented crystal structure, as compared to the random arrangement in the unstretched mass, so that the relative hardness of

the filament cannot be determined by computation from tests made upon the mass.

Slurries are formed therewith containing about 20 percent of the indenting particles, noting that the proportions may be modified within the limits of having a slurry which is too thick to enter between the fibers during the preliminary loading operation, or one which is so thin that it drains away without depositing the particles ready for operation. The vehicle for the slurry can be selected from a wide range of liquids which are inert relative to the nylon. Water is a cheap and desirable vehicle for materials insoluble therein, such as calcite, glass, diatomaceous earth: and can be used with water-soluble materials such as rocksalt, sodium bicarbonate, or the like, in the form of a saturated solution of the material being used.

The solids content of the slurry, for optimum effect, varies with the material used, the particle size, and the vehicle. In general, it should be in the range of 8 to 20 percent. With diatomaceous earth, a slurry of 12.5 percent by weight in water is satisfactory, and therewith in the illustrative example about 20 percent of the material, based on yarn weight, is taken up by the yarn: the particles tend to be filtered out by the yarn and remain enmeshed in the skein, while the water is squeezed out. A general range of 8 to 16 percent in a water slurry is preferred for diatomaceous earth, noting that with less than 8 percent, the dulling action is very slow, while more than 16 percent may cause an uneven treatment as the water vehicle is squeezed out and the presence of an excess of material in the skein leads to matting and a low amount of relative movement. With silica and non-friable materials, enmeshing was more regular and more than 40 percent could be present in the slurry, with a preference for 20 to 40 percent.

During use of the material, it has been found that the presence of a greater amount of particles, other conditions being constant, will give a greater dulling effect up to the 40 point at which the total mass is relatively stiff and corresponds to the yarn fibers being embedded within an essentially solid mass of particles so that little relative movement of the fibers can occur.

Using a silica powder, commercially designated as passing a 325 mesh screen, in determining the effects of the sizes thereof, it was found upon microscopic examination, the original powder exhibited a few particles as large as 40 microns. When such a powder was fractionated by repeated settling, an intermediate fraction was more effective than the smaller sized fractions. Fractions were used in dulling experiments, using 20 percent by weight of the dry yarn, sprinkling evenly over the wet yarn and distributing by working with the hands. The working 55 time was 15 minutes. The results were as follows:

Table I

| Particle |             | Visual Dulling | Reflectance Values—White Yarn |         |       |         |
|----------|-------------|----------------|-------------------------------|---------|-------|---------|
|          |             |                | Parallel                      | Perpen- | Ratio | Percent |
| Sample   | Size        |                |                               |         |       | Drop    |
| Control  |             |                |                               |         |       |         |
| 1        | less than 5 | least          | 0.67                          | 0.92    | 1.37  |         |
| 2        | 3-7         | more than 1    | 0.71                          | 0.85    | 1.20  | 12.4    |
| 3        | 10-15       | more than 2    | 0.71                          | 0.84    | 1.18  | 12.6    |
| 4        | 20-25       | same as 3      | 0.72                          | 0.84    | 1.17  | 12.6    |

NOTE.—The "reflectance values" are those determined as set out below, as a preamble to Table III.

Table I-A

| Particle | Visual Dulling | Reflectance Values—Black Yarn |         |       |              |
|----------|----------------|-------------------------------|---------|-------|--------------|
|          |                | Parallel                      | Perpen- | Ratio | Percent Drop |
| Sample   | Size           |                               |         |       |              |
| Control  |                |                               |         |       |              |
| 1        | less than 5    | least                         | 0.0055  | 0.17  | 30.9         |
| 2        | 3-7            | more than 1                   | 0.0068  | 0.14  | 20.6         |
| 3        | 10-15          | more than 2                   | 0.010   | 0.13  | 13.0         |
| 4        | 20-25          | same as 3                     | 0.010   | 0.13  | 13.0         |
|          |                |                               |         |       | 57.9         |
|          |                |                               |         |       | 57.9         |

The size for Samples 1-4 is stated in microns. Microscopically examined, Sample 4 contained some particles as large as 40 microns and a few as small as 15 microns. Samples 2 and 3 were quite uniform.

A powdered calcite, designated commercially as having an average large particle size of 25 microns, was more effective than one with an average size of 5 microns in work upon nylon fibers which were 10 denier or over. Upon microscopic examination, the 25 micron material was found to have some particles as large as 100 microns but most were in the 10-60 micron range. The material was fractionated by settling; for a fraction A with most of the particles in the range of 10 to 30 microns, and a fraction B in the range of 40 to 60 microns with some particles as large as 100 microns. It was employed as with the silica powder. Some grinding of the calcite occurred during the dulling: but many large particles still remained. The two fractions gave essentially the same result, with values of 0.73 for parallel-plane viewing and 0.84 for perpendicular-plane viewing of the undyed specimens: no tests were made with dyed yarn. These values represent a change of ratio from 1.37 in the control to 1.15 of the treated material, with a percentage drop of 16. Thus, the results are comparable with those for silica powder as set out in Table I.

In further experiments, a residue from the glass polishing industry was used (commercially available by the name Gartex). This material consists of silica and glass particles, but contains some particles larger than those with the silica described above: the results are comparable. Being commercially designated as having a particle size of 25 microns, it was fractionated by repeated settling in water. Fraction A contained particles largely between 5 and 10 microns, a few being as large as 15 microns and some smaller than 5 microns. Fraction B was quite uniform in the range of 20 to 30 microns. Fraction C was largely particles above 60 microns, some being as large as 100, while a few were as small as 20. Single skeins were run for 15 minutes. Fraction B gave better results than fractions A or C. Fraction A was least effective. There was no conclusive evidence of damage to the yarn even with fraction C, where particles were larger than the diameters of the yarn itself. The pressure was increased, by employing a metal sleeve with a thin rubber tubing over one of the lower rollers. The skein was confined in a space an inch and a half wide. The dulling effect with fraction C was definitely better than at the lower pressure, being somewhat greater than that obtained with fraction B at the lower pressure. A portion of the yarn was knitted into fabric and dyed: there was no stitch distortion or uneven dyeing as would be present in damaged yarn. A test of breaking strength showed about 7 percent loss. The samples were compared visually with the samples of Table IV below, as

signing arbitrary dullness values of 1, 2 and 3 to the 10, 15 20 and 30 minute samples. The results were:

Table II

| Sample | Particle Size               | Dullness Value  |
|--------|-----------------------------|-----------------|
| 1      | 5-10 microns                | 2 $\frac{1}{4}$ |
| 2      | 20-30 microns               | 2 $\frac{3}{4}$ |
| 3      | 40-60 microns               | 1 $\frac{1}{4}$ |
| 4      | 40-60 microns—High pressure | 3               |

To determine the effect of large particles, an emery powder was employed having particles in the range of 300 microns with a few having a dimension as great as 500 microns. Single skeins were run under the conditions described for the machine above, and then under increased pressure by use of the metal tube with the thin rubber sleeve. Very little dulling effect was observed at the lower pressure, but at the higher pressure a fair dulling occurred but with a great deal of damage. Upon examination, the fiber was grossly distorted in many places. In some places it was flattened, and at many spots it was completely broken or cut through.

Thus, the optimum particle size is somewhat dependent upon the pressure employed. With the stated pressures of around 1000 pounds in the described machine, the optimum particle size is around 20 microns for non-friable materials when 15 denier nylon is being treated: with a preferred range of 10 to 30 microns with filaments of 10 to 80 micron diameter. The maximum size of particles, to avoid damage, appears around 150 microns for uses up to 70 denier. In operation, there appears no advantage in the use of the larger particles, and there is some difficulty with them as slurries tend to settle very rapidly and are more difficult to apply uniformly and remove completely.

The diatomaceous earth is a composite of shells and fragments of disk and needle shape, with disks up to 100 microns diameter and needles up to 150 micron length and 5-20 micron diameter. In practice therewith, it has been noted that, while the original material settled rapidly in water, the spent slurry after a first indenting operation was much slower in settling, indicating that the individual shells had broken during the operation, thus affording many sharp edges, a conclusion supported by microscopic examination. The commercial material employed is designated as having an average particle size of 7-9 microns, but microscopic examination has indicated the above range.

There are relationships between the unit pressure upon the nylon filaments and between the amount of indenting material present, and the largest permissible size for optimum effects. Assuming that the fibers are cylinders of the same size, and parallel and closely packed, the area of unoccupied space in a cross-section is about 10 percent of the area occupied by the fibers. A spherical particle of  $\frac{1}{6}$  the diameter of a filament, if placed in a space, will touch the surrounding filaments and represents a maximum dimension which in the assumed case causes no filament displacement. On the quantity basis, tightly packed powdered silica has a density of about 1.5 times that of nylon, so that the 10 percent voids can receive powdered silica up to about 15 percent of the weight of

the nylon. Upon compression, in either case, the filaments are distorted by the sphere or upon peripheral edges and corners of the silica particles. With the sphere, the distorted area is so large that no appreciable change of light reflection is apparent later, but with the silica particles, the disturbances are smaller and more numerous, so that a dulled effect results. With extremely small particles, and close indentations by their edges and corners, the shining or mirrorlike surface appearance is replaced by a sheen, noting that very fine abrasives are used to 10 polish optical lenses of glass.

The pressure employed is distributed by the rollers over the skeins and the individual filaments. It has been found that the pressure can be practically determined for optimum effects upon the basis of the number of skeins present. In the illustrative machine, with 24 skeins of 2 ounces each, and 4 inch rollers, a total pressure of 500 pounds gives much less effect in 21 minutes than 1000 pounds in 10½ minutes.

The above illustrative example, with a total cycle of 15 minutes, was effective with 15 denier monofilament yarn. By comparison, a 12 denier monofilament yarn was successfully treated to a like dullness with the same timing for the later operations but with 15½ minutes employed in the first step of working with the indenting particles.

It may be stated, generally, that with proper pressure the dulling effect is rapid at first and then increases more slowly. With the instance of 15 denier yarn in a 15 minute cycle including action in the presence of the indenting material for 10½ minutes, to give a commercially acceptable appearance, an increase to 20 minutes in the dulling sub-cycle gives a greater effect, while an increase to 30 minutes for the sub-cycle gives only a slight further effect, other conditions being kept the same. A 2 ounce skein contains over 10 miles of yarn; the treatment for 10½ minutes causes far less than one break per skein during the subsequent unwinding—a result in which the frequent reversals appear a great factor.

In an illustrative machine, the rollers 45, 71 and 87 were 24 inches long, and 24 skeins, each of 2 ounces of nylon, occupied 22 inches between the outer guide fingers 105, being grouped 4 skeins between each two successive fingers. The housing was about 8 inches between the door 28 and the back wall 26 and about 30 inches high from the lower edge to the lower ends of the tension spring pipes 35. The lower pressure rollers 45, 71 were each 4 inches in external diameter, with a flexible rubbery covering (the material commercially available under the trade name neoprene, Shore A durometer test 55-60, is satisfactory) about ¼ inch thick. The upper tension roller 85 was made of aluminum and 3 inches in diameter. The axis of the lower pressure roller 45, in the absence of yarn, was about 23 inches below the top of the housing. When in operating position, the axis of the pressure and tension rollers and of the spray pipe 99 were in a vertical plane located about 6 inches from the rear wall 26. In this machine, the lever arms 43 supported the lower roller 45 with its axis about 3½ inches from the fulcrum point 42, and the total weight acting on the rear end of arms 43 was about 200 pounds at a fulcrum distance of about 16 inches, thus representing a pressure of about 1000 pounds at the lower pressure roller 45, or about 45 pounds per effective inch of length of this roller.

In the above description of results, stated as occurring with increased pressure, the effect corresponded to about an eight-fold increase.

Other practices, for example with 40 denier monofilament yarn and 70 denier 34 filament yarn, have produced good dulling effects respectively in 10 minutes and 15 minutes under the pressure and other conditions stated above for the illustrative machine and practice.

The operation is one of indentation rather than abrasion and removal of material. Weight studies upon the yarn, comparing weights before and after treatment, indicate that very small losses occur from the fibers and fila-

ments. Likewise, strength trials indicate that there is a maximum reduction in tensile strength (6 inch pieces) of 5 percent. The values of strength vary from skein to skein as received from the manufacturer, and the observed differences are well within the range. Optically, at low magnification, the fiber surfaces have an appearance as though blasted with very fine sand; at higher powers and in a dark field, small light arrows appear and are believed to indicate the great irregularity of the surface. Using the preferred siliceous particles, the product had the scroopy feel of silk.

The dulling effect can be numerically measured by a reflectance meter, most suitably with the yarn dyed black and by comparison to an untreated yarn. The samples 15 should be thoroughly clean, and made into skeins of parallel threads, or better into seriplane panels (on dull black cardboard as a background) containing for example with 15 denier nylon at least 800 threads per inch, and corresponding numbers of threads for other deniers. 20 For accuracy, the background and the number of threads per inch should be the same for the control and the treated specimens. Employing a Welch Densichron device with a 45 degree reflectance head, which was adjusted and calibrated for reflectance values in the gray scale of 25 I.C.I. "y" tristimulus values for illuminant "C," based on measurements with the G.E. recording spectrometer, the standards were small test pieces, with one side glazed and the other side unglazed, varying from white through various shades of gray to black. In use, a light beam strikes the sample at an angle of 45 degrees: light which is reflected as from a plane mirror is not measured, and a perfect plane mirror would give a zero reading. Light which is scattered or deflected is read by the electric photometer at an angle of 90 degrees. The effect differs 30 according to the angle of the plane of the beam: when the beam plane is perpendicular to the axes of the threads, the values for dulled yarn are less than for the control; when the beam plane is parallel, the values for dulled yarn are greater than for the control. The apparatus used was constructed to operate at three scales of sensitivity, a decimal related: the difference between untreated yarn and dulled yarn was apparent at a coarse setting, while the differences between yarn treated for 20 and 30 minutes required resort to a more sensitive scale.

In general, it was found that the values (black-dyed specimens) with parallel light increased up to 250% upon dulling treatment under commercially satisfactory conditions; an increase of 25 percent is a minimum for practical purposes; with values of increase of 50 to 150 percent representing desirable and sufficient effects. Correspondingly, with perpendicular light, the same specimens showed decreases up to 70 percent: a 20 percent decrease is required for commercially useful effects; decreases of 25 to 50 percent representing desirable and sufficient effects. The change of ratios of readings with parallel and with perpendicular light, for the control and for the treated specimens, is particularly characteristic.

In general, the ratio for the treated yarn should be at least 15 percent and preferably 30 percent less than with the control: ratio changes as high as 90 percent have been observed. The ratio decreases with the duration of treatment, other factors being the same, but is not linear with time. With black-dyed specimens, in seriplane panel tests, at least a 10 percent drop of the ratio, compared with the control, is required for commercially useful effects: with white (undyed) skein specimens, the drop of ratio should be 10 to 70 percent for commercially useful effects; and, with black-dyed skeins, at least 25 percent.

It may be remarked that nylon itself usually contains a pigment as dulling or opaques agent, often white. When tests were made with such light-colored yarns (sometimes called "dull" or "semi-dull" according to the amount of pigment present), the general illumination effect tends to obscure the results. For instance,

by mounting seriplane panels on a black cardboard, with 2400 threads of 15 denier per inch, results were obtained with white yarn:

Table III

|                         | Light Beam Plane |         | Ratio | Percent Drop of Ratio | 5 |
|-------------------------|------------------|---------|-------|-----------------------|---|
|                         | Parallel         | Perpen- |       |                       |   |
| Control.....            | 0.67             | 0.92    | 1.37  |                       |   |
| 10 minutes dulling..... | 0.72             | 0.87    | 1.21  | 11.7                  |   |
| 20 minutes dulling..... | 0.76             | 0.86    | 1.13  | 17.6                  |   |
| 30 minutes dulling..... | 0.77             | 0.83    | 1.08  | 21.1                  |   |

Noting that the light perceived by the apparatus depends upon the color of the specimens, the following results of tests with 15 denier white semi-dull nylon, untreated (control) and treated for 10, 20 and 30 minutes with diatomaceous earth are indicative, the samples being made up into small skeins containing 800 fibers each, with one lot tested in the original color (white) and another lot tested after dyeing black:

Table IV

|                 | Dyed Black     |              |                     |              | Ratio | Percent Drop of Ratio | 30 |  |  |  |
|-----------------|----------------|--------------|---------------------|--------------|-------|-----------------------|----|--|--|--|
|                 | Parallel Light |              | Perpendicular Light |              |       |                       |    |  |  |  |
|                 | Rdg            | Percent Inc. | Rdg                 | Percent Dec. |       |                       |    |  |  |  |
| Control.....    | 0.0060         |              | 0.18                | 22           | 30    |                       |    |  |  |  |
| 10 minutes..... | 0.0075         | 25           | 0.14                | 22           | 19    | 36.7                  |    |  |  |  |
| 20 minutes..... | 0.013          | 116          | 0.13                | 28           | 10    | 66.7                  |    |  |  |  |
| 30 minutes..... | 0.016          | 166          | 0.09                | 50           | 5.6   | 81.0                  |    |  |  |  |

"Rdg" signifies the apparatus reading; "Percent Inc." the percentage increase of reading over that for the control; "Percent Dec." the corresponding percentage decrease; and "Percent Drop of Ratio" the percentage drop from the ratio found for the control specimen.

Table IV-A

|                 | White Samples (undyed): coarse scale |              |                     |              |       |                       | 55 |  |
|-----------------|--------------------------------------|--------------|---------------------|--------------|-------|-----------------------|----|--|
|                 | Parallel Light                       |              | Perpendicular Light |              | Ratio | Percent Drop of Ratio |    |  |
|                 | Rdg                                  | Percent Inc. | Rdg                 | Percent Dec. |       |                       |    |  |
| Control.....    | 0.87                                 |              | 1.2                 | 22           | 1.4   |                       |    |  |
| 10 minutes..... | 1.0                                  | 14.7         | 1.2                 | 0            | 1.2   | 14.3                  |    |  |
| 20 minutes..... | 1.1                                  | 16.1         | 1.2                 | 0            | 1.1   | 21.4                  |    |  |
| 30 minutes..... | 1.1                                  | 16.1         | 1.1                 | 8.3          | 1.0   | 28.6                  |    |  |

These results are comparable to those of Table III; noting that Table III is based upon white seriplane panel specimens and Table IV-A on white skeins.

That the result comes from the dulling is shown by performing tests upon nylon which had been dyed blue-black before the treatment, as shown by the following:

Table V

|              | Light Beam Plane |         | Ratio | 70 |
|--------------|------------------|---------|-------|----|
|              | Parallel         | Perpen- |       |    |
| Control..... | 0.010            | 0.17    |       |    |
| Dulled.....  | 0.016            | 0.10    | 17.0  |    |

Further illustrative is the following result, produced by a far-reaching treatment of 15 denier yarn of the so-called "semi-dull" type. Diatomaceous earth was used. 75

75

14  
Table VI

|              | Parallel |              | Perpendicular |              | Ratio | Drop, Percent |
|--------------|----------|--------------|---------------|--------------|-------|---------------|
|              | Rdg.     | Percent Inc. | Rdg.          | Percent Dec. |       |               |
| Control..... | 0.006    |              | 0.17          |              | 28    |               |
| Dulled.....  | 0.022    | 266          | 0.065         | 67           | 3     | 89            |

The treated specimen of Table VI was dulled beyond commercial requirements: wherewith the ratio dropped by 89 percent.

Tests made with so-called "bright" commercially available yarn, which contained no pigment, and was of 70 denier size, gave the following result on meter readings of small skeins containing 200 threads.

Table VII

|                    | Parallel |              | Perpendicular |              | Ratio | Percent Drop |
|--------------------|----------|--------------|---------------|--------------|-------|--------------|
|                    | Rdg.     | Percent Inc. | Rdg.          | Percent Dec. |       |              |
| Control-white..... | 0.60     |              | 2.7           |              | 4.5   |              |
| Sample-white.....  | 0.85     | 25           | 1.7           | 37           | 2.0   | 55.6         |
| Control-black..... | 0.005    |              | 0.13          |              | 25    |              |
| Sample-black.....  | 0.010    | 100          | 0.10          | 30           | 10    | 61.5         |

The values indicate that the effect has occurred, and the results with the dyed specimens are parallel to those obtained with so-called semi-dulled yarns.

The results in the tables show that apparatus can be employed in determining the existence of the effects and the regular course of the treatment; and show the possibility of specifying the treatment effect to be attained. In actual practice, visual comparison can readily be made by a person skilled in the work, by merely viewing seriplane panels with proper lighting. Comparisons of specimens thus made agree well with apparatus measurements.

A further manner of determining the effects of the treatment is by comparison of the rate of acceptance of dye after successive stages of treatment, with use of the reflectance meter and its gray scale of standards. When the dulled yarn and an undulled control were dipped for 5 minutes at 100 degrees F. in a 0.1 percent solution of a black dye (Glycolan Black B), then washed well with soap, and dried, the observed results are definite and reproducible. Illustrative of this is the following, representing results obtained with a parallel beam:

Table VIII

|                 | Reading-Parallel | Percent Change |
|-----------------|------------------|----------------|
| Control.....    | 0.50             |                |
| 10 minutes..... | 0.44             | 12             |
| 20 minutes..... | 0.40             | 20             |
| 30 minutes..... | 0.36             | 28             |

Since the values in Table VI are based upon material of like history, the variance in dyeability by heat treatments and other prior history of the nylon yarn is excluded.

The difference in the effect of dulling in the present manner and that by incorporating pigment into the filaments for absorbing or scattering light, can be illustrated by the behavior upon dyeing. When the so-called dulling is attained by incorporated pigment, the effect is essentially lost when the filaments are dyed black, because the surface luster has not been changed: but with yarns treated in the present fashion, the effect is more striking after dyeing to very deep shades.

The effects upon the yarn are the production of an increased rate of dyeing, a change in the feel of the yarn to produce a scroopy hand, a decreased coefficient of

friction toward smooth surfaces such as porcelain guides, along with the decrease in gloss or luster.

The variables which dominantly control the rate and effect of the treatment upon a given fibrous material are (1) the indenting material employed, by composition, amount, and particle size; (2) the pressure employed; and (3) the duration of treatment.

There is a correlation between the pressure and time, but the relationship is not inversely linear. For example, with a force of 500 pounds upon the rollers of the described machine, there was little dulling in 10 minutes and a multiple of this time is required to attain a satisfactory effect: a satisfactory dulling was attained in 10 minutes with a force of 1000 pounds, whereas 750 pounds gave a somewhat lesser effect. These values correspond to pressures of 20, 30 and 40 pounds per inch of length of the rollers, or per skein of yarn.

The change in dyeing properties is indicated by the behavior with acetate dyes, in which the maximum change of rate appears to occur before the maximum dullness is reached.

It will be understood that the illustrative practice of the invention is not restrictive: and that the same may be employed in many ways within the scope of the appended claims.

What is claimed is:

1. The method of dulling nylon and like fibers which comprises supplying a finely divided moistened indenting material into a mass of the fibers, passing the total mass between pressure rollers, at least one said roller having a resiliently yielding surface whereby to procure a kneading action of the fibers and indenting material, and repeating the passage until the surfaces of the fibers have received indentations over their areas.

2. The method of dulling nylon and like fibers which comprises supplying a slurry of finely divided indenting material to and into a mass of the fibers, passing the total mass between pressure rollers, at least one said roller having a resiliently yielding surface whereby to procure a kneading action of the fibers and indenting material, and repeating the passage with alternation of the direction of passage from time to time until the surfaces of the fibers have received indentations over their areas.

3. The method of dulling nylon and like fibers in skeins, which comprises supplying a slurry of finely divided indenting material to the fibers in the skein, stretching the skein loop over a first pressure roller, applying pressure to the fibers in the loop by coaction of a second pressure roller with said first pressure roller, at least one of said pressure rollers having a yielding surface whereby a kneading and relative displacement of the fibers is produced, rotating one of the pressure rollers successively in alternative directions, and continuing the pressure and alternative rotation until the surfaces of the fibers have received indentations over their areas.

4. The method as in claim 3, including the step of delivering a rinsing liquid upon the skein loop while stretched over the first pressure roller and while continuing the alternate rotation.

5. The method as in claim 3, including the steps of successively delivering firstly a wetting liquid, secondly a soap solution, and thirdly a rinsing liquid upon the skein loop while stretched over the pressure and tension rollers and while continuing the alternate rotation.

6. The method as in claim 3, in which the indenting

material comprises sharp particles of material harder than 2 on the Moh scale, and present as a slurry having a solids content of 8 to 40 percent, the particles being substantially within the range of 3 to 150 microns.

5 7. The method as in claim 6, in which the indenting material is diatomaceous earth.

8. The method as in claim 6, in which the indenting material is a silica powder.

9. The method as in claim 6, in which the indenting material is a calcite powder.

10 10. The method as in claim 6, in which the indenting material is a glass-polishing residue of silica and glass particles.

11. The method as in claim 3, in which the pressure is about 45 to 360 pounds per effective inch of length of a pressure roller.

12. The method of dulling nylon and like fibers in skeins, which comprises kneading the fibers of a skein loop between yielding roller surfaces under a pressure of

20 45 to 360 pounds per effective inch of length thereof, in the presence of a slurry of finely divided indenting material enmeshed with the fibers, and continuing the kneading for effecting indentation in the substantial absence of removal of surface material from the fibers, until the 25 light reflectance value has increased at least 25 percent under parallel light.

13. The method of dulling nylon and like fibers in skeins, which comprises kneading the fibers of a skein loop between yielding roller surfaces under a pressure of 30 45 to 360 pounds per effective inch of length thereof, in the presence of a slurry of finely divided indenting material enmeshed with the fibers, and continuing the kneading for effecting indentation in the substantial absence of removal of surface material from the fibers, until the 35 light reflectance value has decreased at least 20 percent under perpendicular light.

14. The method of dulling nylon and like fibers in skeins, which comprises kneading the fibers of a skein loop between yielding roller surfaces under a pressure of 45 to 40 360 pounds per effective inch of length thereof, in the presence of a slurry of finely divided indenting material enmeshed with the fibers, and continuing the kneading for effecting indentation in the substantial absence of removal of surface material from the fibers, until the 45 ratio of reflectance values for parallel and for perpendicular light has changed at least 15 percent relative to said values with the untreated fibers.

References Cited in the file of this patent

UNITED STATES PATENTS

|           |                     |               |
|-----------|---------------------|---------------|
| 1,890,643 | Ellis et al. -----  | Dec. 13, 1932 |
| 1,957,508 | Taylor -----        | May 8, 1934   |
| 2,077,283 | Taylor et al. ----- | Apr. 13, 1937 |
| 2,251,508 | Watson -----        | Aug. 5, 1941  |
| 2,322,094 | Newhard -----       | June 15, 1943 |
| 2,325,060 | Ingersoll -----     | July 23, 1943 |
| 2,505,033 | Elvin et al. -----  | Apr. 25, 1950 |
| 2,561,133 | Petkewicz -----     | July 17, 1951 |
| 2,592,161 | Lorig -----         | Apr. 8, 1952  |

FOREIGN PATENTS

|         |                     |                |
|---------|---------------------|----------------|
| 335,204 | Great Britain ----- | Sept. 15, 1930 |
| 556,252 | Great Britain ----- | Sept. 27, 1943 |
| 713,276 | Great Britain ----- | Aug. 11, 1954  |
| 737,928 | France -----        | Oct. 10, 1932  |